

## UNITED STATES PATENT OFFICE

1,951,091

METHOD OF MANUFACTURING CHROMIUM  
OF CHROMIUM ALLOYS

Ture Robert Haglund, Stockholm, Sweden

No Drawing. Application January 23, 1933, Serial  
No. 653,185. In Sweden August 22, 1932

7 Claims. (Cl. 75—48)

This invention relates to processes of manufacturing chromium or chromium alloys, such as ferro-chrome low in carbon and chromium-alloyed iron and steel, in an electric furnace in which a refining action is obtained by means of a molten slag bath containing chromium oxide, and especially to such processes in which chromiferous material is successively supplied to the slag bath in the form of a pulverized chromium alloy high in carbon, for instance a pulverized ferro-chrome containing 60 to 75% Cr and 6 to 10% C. A process of this kind is described in my copending application Ser. No. 632,865 filed September 12, 1932. Said application describes 15 a process for decarburizing chromium alloys by reaction with a slag bath having a high content of chromium oxide and being heated by means of electrodes operating in electrical connection with the top portion of said slag bath, fine particles of a chromium alloy high in carbon being successively added to the slag bath and spread therein on account of the stirring action caused by the carbon monoxide evolved in the slag by the reaction between the chromium oxide of the slag 20 and the carbon of the added particles of chromium alloy.

The chief object of the invention is to maintain a high content of chromium oxide in the slag bath during the whole operation, thus facilitating the refining action on the chromiferous material supplied to the slag bath.

According to the invention the chromium alloy, is more or less completely roasted or oxidized before it is supplied to the slag bath. In this manner a material rich in chromium and chromium oxide but substantially free from other oxides, such as aluminium and magnesium oxides, having a diluting action on the slag, is supplied to the slag bath, whereby the latter in spite of the 35 reducing action of the carbon of the chromium alloy, can be maintained at a high percentage of chromium oxide during the whole refining operation.

It is, however, possible to supply a part of the 40 chromium oxide required for the process in the form of chromium ore or to produce a part of the chromium oxide by oxidation of a part of the metallic chromium in connection with the refining operation, for instance by additions of 45 iron ore.

It is not necessary to preoxidize all chromium 50 alloy used as charging material in carrying out the process as it will be sufficient to oxidize only a part thereof, in which case the oxidation, however, is carried comparatively far, if desired to

complete oxidation. Generally, it is, however, more suitable to oxidize partly the chief part of the chromium alloy or the whole alloy so that the particles of chromium alloy to be supplied to the slag bath are coated by a shell of chromium oxide. Such particles do not attract the electric current flowing from the electrodes to the slag bath and accordingly volatilizing of metallic chromium is avoided which otherwise takes place by the direct action of the electric current or the electric arc on alloy particles having clean metallic surfaces. Furthermore, the current flow will be more quiet when using an alloy the particles of which have a protecting surface layer of oxide and the absorption of nitrogen in the alloy which easily takes place when an electric arc is playing against non-oxidized surfaces of the chromium alloy particles, will also be avoided.

The roasting or oxidation of the ferro-chrome 75 is carried differently far, dependent on the alloy to be manufactured. If a ferro-chrome with a content of carbon less than 0.5% shall be manufactured a degree of oxidation amounting to 15 to 40% should be used, whereby it will be possible to 80 maintain a chromium oxide content in the slag bath of about 50 to 80% Cr<sub>2</sub>O<sub>3</sub>. In manufacturing chromium-alloyed iron, for instance of the rustless qualities, it is possible to work with essentially lower degrees of oxidation, for instance 85 between 5 and 15%, and even lower, as the composition of the slag bath in such case can be regulated also in other manner, for instance by additions of iron ore. Additions of other alloying metals, for instance nickel, can in such case 90 be supplied either to the metal in the electric furnace or partly or wholly after the tapping of the alloy from the electric furnace. In manufacturing chromium-alloyed iron or steel an adjustment of the percentage of chromium of the 95 alloy produced can also be effected by adding ferro-chrome low in carbon after the alloy has been tapped from the furnace.

The roasting or oxidation of the chromium alloy may be performed by means of atmospheric air, oxygen, steam or other oxidizing agent and is carried out, preferably, at temperatures between 1200 and 1400° C. In some cases, especially when a relatively low degree of oxidation is aimed at, a considerably lower temperature can be used, for instance down to 900° C. The roasting of the pulverized ferro-chrome may be facilitated by mixing it with other substances having a loosening action thereon or which promote the forming 100 or chromate, for instance limestone or quick- 110

lime. An addition of 1 to 2% CaO will be sufficient for such purpose. Suitable furnaces for the performance of the roasting operation are, for instance, channel furnaces, rotary furnaces and down-draft pans otherwise used in sintering fine ores. The oxidation process has also a decarbonizing action on the chromium alloy. For instance, at a roasting carried out at 1200° C. to an oxidation degree of 10% a decarbonizing 10 amounting to more than 20% has been noted.

The chromium alloy used as starting material should have a low percentage of silicon, preferably less than 1%. The most favorable results have been obtained with chromium alloys containing only one or some tenths of a percent of Si.

What I claim is:—

1. In a method of manufacturing chromium or chromium alloys by melting and refining a carbonaceous chromium alloy in a molten slag bath containing chromium oxide, the step which consists in partially oxidizing the chromium content of the alloy before adding it to the slag bath.
2. A method of manufacturing chromium alloys low in carbon, which comprises roasting ferro-chrome high in carbon to partially oxidize its content of carbon and partially oxidize its content of chromium, and then melting and refining the roasted ferro-chrome in a molten slag bath containing chromium oxide.
3. A method as claimed in claim 1, in which

the chromium alloy is pulverized and then roasted to an oxidation degree of 5 to 40%.

4. A method as claimed in claim 1, in which a chromium alloy low in silicon is roasted to partially oxidize its content of chromium and then melted and refined in a molten slag bath containing chromium oxide.

5. A method of manufacturing chromium alloys low in carbon, which comprises roasting ferro-chrome high in carbon to partially oxidize its content of chromium in presence of a basic substance which promotes the formation of chromate in the roasting operation, and then melting and refining the roasted ferro-chrome in a molten slag bath containing chromium oxide.

6. A method of manufacturing chromium alloys low in carbon, which comprises roasting ferro-chrome high in carbon to partially oxidize its content of chromium in presence of a basic substance, and then melting and refining the roasted ferro-chrome in a molten slag bath containing chromium oxide.

7. In a method of manufacturing chromium or chromium alloys by melting and refining a chromium alloy having a high content of carbon by means of a molten slag bath containing chromium oxide, the step which comprises adding the chromium alloy at least partially in the form of small particles having a skin of chromium oxide on their surface.

TURE ROBERT HAGLUND.

105

110

115

120

125

130

135

140

145

150